

L. P. BURROWS.

ALLOY FOR FORGING STEEL AND METHOD OF PRODUCING SAME FROM NICKEL ORE.

APPLICATION FILED JAN. 20, 1920. RENEWED SEPT. 22, 1921.

1,424,710.

Patented Aug. 1, 1922.



Inventor

Linus P. Burrows

By Spear, Middleton, Danaher and the  
Attorney

# UNITED STATES PATENT OFFICE.

LINUS PORTER BURROWS, OF ERIE, PENNSYLVANIA; LENAH B. ARCHER EXECUTRIX  
OF SAID L. P. BURROWS, DECEASED.

## ALLOY FOR FORGING STEEL AND METHOD OF PRODUCING SAME FROM NICKEL ORE.

1,424,710.

Specification of Letters Patent.

Patented Aug. 1, 1922.

Application filed January 20, 1920, Serial No. 352,775. Renewed September 22, 1921. Serial No. 502,548.

*To all whom it may concern:*

Be it known that I, LINUS PORTER BURROWS, a citizen of the United States, and resident of Erie, Pennsylvania, have invented certain new and useful Improvements in an Alloy for Forging Steel and Method of Producing Same from Nickel Ore, of which the following is a specification.

In an application filed by me August 7, 10 1915, renewal No. 335,107, I have described the treatment of nickel ore whereby I obtain a new product disintegrated by exposure to air. This is particularly adapted for use after further treatment as an alloy in the 15 production of forging steel.

I perceived that in order not to break up the molecule of steel so that it would not forge, I must reduce the chemical strength of the former product of my application 20 aforesaid in order to produce an alloy for forging steel and to this end I subject the product of my former application to heat, with the result that I reduce its chemical strength to the point required. This I accomplish without appreciably oxidizing the 25 product.

This treatment I carry out preferably in a furnace such as shown in the accompanying drawing in which Fig. 1 is a side elevation, Fig. 2 a horizontal section; Fig. 3 a cross section and Fig. 4 an end view.

The furnace has a bottom A with crown B, a flue C, and doors D closing the front opening. I provide a false bottom E divided by lateral partitions e, and into the spaces formed by these partitions project gas pipes f, extending from a header or main F. The gas pipes are alternately arranged so that the flame comes in at one side of one compartment while the other compartment is supplied by a jet from the opposite side. Openings e' are provided opposite the position of the burners to allow for the exit of the products of combustion, 45 and upon the false bottom I place the powder which is subjected to a low red heat approximately between 1200° and 1600° F., resulting in a reduction of the weight of the previously recovered product approximately 50 20% by evaporation.

I find that by actual tests by the use of from one to two per cent of my alloy I am able to produce a forging steel equal in tensile strength and surpassing in many other useful qualities present steel produced by 55 the use of three and one-half per cent metallic nickel.

It will of course be understood that I use in the production of the alloy of the present application the process particularly described in my application No. 335,107, namely, the ore containing nickel is crushed and heated for five or six hours in the presence of the gaseous product of my Patent No. 680,313. The resulting product is then removed 60 from its container and smelted in a crucible. The slag is removed and the remaining metallic product broken up and exposed to the atmosphere until perfect disintegration takes place, usually from 12 to 24 hours, depending upon the size of the lumps. This results in a brownish black powder which forms the basis of the product of this application.

I have found by the actual carrying out 75 of the invention that the product of my former application comprising a very fine brownish black powder, must be further treated in order to produce my alloy for the production of a forging steel, and this treatment consists in subjecting the said product to evaporating action at a low red heat without material oxidization, and that this treatment results in a new product which is 80 in the form of a purplish powder. 85

What I claim is:

1. The herein described process consisting in subjecting crushed nickel ore to the action of a gaseous product in a closed chamber until the oxygen is removed from the ore, 90 subjecting said treated and refined nickel ore to a smelting process; breaking up the metallic product and disintegrating the same by exposing it to the atmosphere, taking the disintegrated material and subjecting it to 95 an evaporating action at a low red heat without material oxidization resulting in the reduction of the weight of the air disintegrated product approximately twenty per cent.

2. The herein described process consist- 100

ing in subjecting crushed nickel ore with flux additions to a smelting process; the metallic product disintegrating on exposure to the atmosphere; taking the disintegrated material and subjecting it to heat, resulting in the reduction of the weight of the disintegrated product.

3. An improved article of manufacture produced from nickel ore in the form of a purplish powder and adapted for use as an alloy for steel.

In testimony whereof, I affix my signature.

LINUS PORTER BURROWS.